

## UNITED STATES PATENT OFFICE

2,575,195

DIBASIC ACID ESTERS AND METHOD FOR  
PRODUCING THEMPaul V. Smith, Jr., Westfield, N. J., assigner to  
Standard Oil Development Company, a corpo-  
ration of DelawareNo Drawing. Application October 1, 1948,  
Serial No. 52,428

8 Claims. (Cl. 260—485)

1

This invention relates to a new class of compounds which have been found to be particularly suitable for use as synthetic lubricants because of their low pour points and high viscosity indices.

In the lubricant art, considerable progress has been realized in recent years in the production of lubricants characterized by one or more specific properties and adapted for particular uses. In the main, this progress can be attributed to two developments: the first, new refining procedures, and the second, addition agents capable of imparting particular properties to available lubricants. Thus, viscosity index improvers and pour depressants are added to automotive lubricants to render the lubricants more adaptable to wide changes in temperature conditions, while other agents are added to improve the load carrying properties of a lubricant which is to be employed, for example, under extreme pressure conditions.

Recently, in an effort to obtain superior lubricants endowed with specific and superior characteristics, a new field has been explored, namely the synthesis of lubricants from various materials. Esters represent one class of materials which have attracted unusual interest as synthetic lubricants. In general, they are characterized by higher viscosity indices and lower pour points than mineral oils of corresponding viscosity. The esters described in the present specification have been found to exhibit very low pour points and high viscosity indices. Lubricants possessing such properties are of special value in the lubrication of engines which are subjected to high temperatures such as combustion turbine engines, particularly those of the "prop-jet" type. Mineral oil lubricants containing added viscosity index improvers, thickeners or other highly non-volatile additives are undesirable for use in such engines because of the tendency to leave a residue which accumulates and interferes with the operation of the engine. A synthetic lubricant of the type described in the present specification is especially adapted to use under such conditions, since the lubricant contains no additives and thus tends to leave no residue upon volatilization.

The new compounds of the present invention which have been found to be particularly suitable for use as lubricating oils are complex esters prepared by reacting one mol of a dibasic acid with one mol of a glycol in such a manner that a half ester is formed, after which the terminal hydroxyl and carboxyl groups are esterified with a mono-basic acid and monohydric alcohol, respectively.

2

More precisely, the new class of compounds may be defined by the following general formula:



where R is an aliphatic hydrocarbon radical, straight chain or branched, saturated or unsaturated, containing 0 to 26 carbon atoms, or it may be an organic radical consisting of a series of saturated aliphatic hydrocarbon radicals linked by one or more atoms of oxygen or sulfur, or both oxygen and sulfur, provided there are at least two carbon atoms between each pair of oxygen or sulfur atoms, and provided further that the total number of carbon, oxygen and sulfur atoms is from 3 to 80 and the total number of sulfur atoms is not greater than 2. R' of the formula represents a glycol radical and may consist of a saturated aliphatic hydrocarbon group, straight chain or branched, containing 2 to 18 carbon atoms, or it may be a series of saturated aliphatic hydrocarbon radicals linked by oxygen or sulfur atoms, or by both oxygen and sulfur atoms, provided there are at least two carbon atoms between each carboxyl group and the nearest oxygen or sulfur atoms and at least two carbon atoms between each oxygen or sulfur atom in the chain, and provided further that the total number of carbon, oxygen and sulfur atoms in the entire R' radical is from 5 to 80 and the number of sulfur atoms is not greater than 2. R'' of the formula represents a monohydric alcohol residue which may be a saturated or unsaturated aliphatic hydrocarbon radical, either straight chain or branched, containing 1 to 20 carbon atoms, or it may be a series of saturated aliphatic hydrocarbon radicals, straight chain or branched, interlinked by oxygen or sulfur atoms, or both oxygen and sulfur atoms, the total number of carbon, oxygen and sulfur atoms being from 4 to 20. The maximum number of oxygen or sulfur atoms or both in the radical R'' is not greater than 5, and there is a chain of at least two carbon atoms between the acid radical and the first oxygen or sulfur atom and a similar chain of at least two carbon atoms between each pair of oxygen or sulfur atoms in the radical. R''' of the formula represents an aliphatic hydrocarbon radical, straight chain or branched, saturated or unsaturated, containing 1 to 22 carbon atoms.

atoms, or it may represent a series of aliphatic hydrocarbon radicals interlinked by 1 to 5 oxygen atoms, there being at least two carbon atoms between each pair of oxygen atoms and at least one carbon atom between the carboxyl group and the nearest oxygen atom, the total number of carbon and oxygen atoms in the radical being from 3 to 22, or it may represent an organic radical consisting of an aliphatic hydrocarbon chain containing a single inter-linked sulfur atom which is separated from the carboxyl group by at least one carbon atom, the total number of carbon and sulfur atoms in the radical being from 3 to 22. The molecular weight of the entire ester should be at least 300 and the viscosity at 210° F. should not be greater than 150 seconds (Saybolt) to provide a product having lubricating properties.

Among the various components of the complex esters of the present invention certain preferences may be pointed out as giving the optimum of desired properties from the standpoint of service as a lubricant. The preferred dibasic acids are the straight chain dibasic acids of the paraffinic group having from 6 to 10 carbon atoms per molecule. The preferred monohydric alcohols are the aliphatic primary alcohols, whether straight chain or branched, containing no oxygen or sulfur atoms and having from 6 to 10 carbon atoms per molecule. The preferred monobasic acids are the fatty acids containing 2 to 10 carbon atoms per molecule.

The complex esters of this invention may be prepared by reacting one molecular proportion of a dibasic acid with one molecular proportion of a glycol under esterification conditions until only one molecular proportion of water of reaction is produced, and thereafter esterifying the unreacted carboxyl and hydroxyl groups with a monohydric alcohol and a monobasic acid, respectively. A method suitable for carrying out the process in detail will be described below in connection with specific examples.

Illustrative examples of the dibasic acids which may be employed in the synthesis of the complex esters of the present invention are the following:

Oxalic acid  
Malonic acid  
Succinic acid  
Glutaric acid  
Adipic acid  
Pimelic acid  
Suberic acid  
Azelaic acid  
Sebacic acid  
Brassylic acid  
Pentadecanedicarboxylic acid  
Tetracosanedicarboxylic acid  
C<sub>4</sub>—C<sub>24</sub> alkenylsuccinic acids  
Diglycolic acid  
Thiodiglycolic acid

The C<sub>4</sub>—C<sub>24</sub> alkenylsuccinic acids listed above are prepared by condensing olefins or mixtures of olefins with maleic anhydride.

The glycols employed in preparing the esters of the present invention include ethylene glycol and any of the paraffinic homologues of the same containing up to 18 carbon atoms. These may include, for example, ethylene glycol, propylene glycol, butylene glycols, pinacone, trimethylene glycol, tetramethylene glycol, pentamethylene glycol, and the like. Since the glycols may also contain oxygen or sulfur atoms, compounds such

as diethylene glycol, triethylene glycol, the polyethylene glycols of the formula



where  $n$  is 1 to 26, and the polypropylene glycols of the general formula



where either R<sub>1</sub> or R<sub>2</sub> is a methyl group and the other is hydrogen, and where  $n$  is 1 to 20, may likewise be employed. Glycols containing sulfur atoms in thioether linkages may also be employed, and these include such compounds as thiadiglycol and 1,2 - bis(2 - hydroxyethylmercapto)ethane. There also may be used glycols containing both oxygen and sulfur in similar linkages; such a compound is bis-[2-(2-hydroxyethoxy)ethyl]sulfide.

The monohydric alcohols employed are typified by the following:

Methyl alcohol  
Ethyl alcohol  
n-Butyl alcohol  
n-Hexyl alcohol  
n-Octyl alcohol  
2-ethylhexyl alcohol  
Cetyl alcohol  
Oleyl alcohol  
Ethylene glycol mono-n-butyl ether  
Ethylene glycol mono-2-ethylbutyl ether  
Ethylene glycol mono-2-ethylhexyl ether  
Ethylene glycol mono-tert-octyl ether  
β-n-Butylmercaptoethanol  
β-tert.-Octylmercaptoethanol  
β-n-Dodecylmercaptoethanol  
Diethylene glycol mono-n-butyl ether  
Diethylene glycol mono-2-ethylbutyl ether  
40 Diethylene glycol mono-2-ethylhexyl ether  
Propylene glycol mono-butyl thioether  
Propylene glycol mono-tert-octyl thioether  
Propylene glycol mono-n-dodecyl thioether  
n-Butylmercaptoethoxyethanol  
45 tert.-Octylmercaptoethoxyethanol  
n-Dodecylmercaptoethoxyethanol  
n-Butylmercaptopropoxypropanol  
tert.-Octylmercaptopropoxypropanol  
n-Dodecylmercaptopropoxypropanol  
50 Propylene glycol mono-n-butyl ether  
Dipropylene glycol monomethyl ether  
Dipropylene glycol monoethyl ether  
Dipropylene glycol mono-n-butyl ether  
Tripropylene glycol monomethyl ether  
55 Tripropylene glycol monoethyl ether  
Tripropylene glycol mono-n-butyl ether  
Propylene glycol monoisopropyl ether  
Dipropylene glycol monoisopropyl ether  
Tripropylene glycol monoisopropyl ether

Many of the above listed ether alcohols, formed by the reaction of ethylene oxide or propylene oxide with aliphatic alcohols, are known in the industry as "Dowanol," "Carbitols," or "Cello-solves."

A group of alcohols especially adapted for use in connection with the present invention are the so-called "Oxo" alcohols, prepared by the reaction of carbon monoxide and hydrogen upon the olefins obtainable from petroleum products. Materials such as diisobutylene and C<sub>7</sub> olefins are suitable for this purpose; also higher molecular weight olefinic materials are sometimes employed. The alcohols obtained in this manner normally have a branched chain structure.

Among the monobasic acids which may be employed in the preparation of the esters of the present invention, the following may be listed as illustrative:

Acetic acid  
Propionic acid  
Butyric acid  
Valeric acid  
Caproic acid  
Caprylic acid

more water collected. The mixture was washed with three 100 ml. portions of saturated sodium carbonate solution and one 100 ml. portion of water. After drying over "Drierite" (anhydrous calcium sulfate) the material was filtered and stripped to a bath temperature of 200-225° C. at a pressure of about 5 mm.

5 The results of tests of various properties of esters prepared by the above general method are  
10 shown in Table I.

Table I

| Component of Ester                                    | Flash Point<br>(° F.) | Kinematic Viscosity |         | ASTM Slope | Viscosity Index | ASTM Pour Point<br>(° F.) |
|-------------------------------------------------------|-----------------------|---------------------|---------|------------|-----------------|---------------------------|
|                                                       |                       | 100° F.             | 210° F. |            |                 |                           |
| Adipic acid                                           |                       |                     |         |            |                 |                           |
| Thiodiglycol                                          | 355                   | 45.720              | 6.950   | 0.707      | 117             | 50                        |
| n-Caproic acid                                        |                       |                     |         |            |                 |                           |
| 2-Ethylhexanol                                        |                       |                     |         |            |                 |                           |
| Adipic acid                                           |                       |                     |         |            |                 |                           |
| Triethylene glycol                                    | 400                   | 38.630              | 7.242   | 0.638      | 143             | >-35                      |
| n-Caproic acid                                        |                       |                     |         |            |                 |                           |
| 2-Ethylhexanol                                        |                       |                     |         |            |                 |                           |
| Adipic acid                                           |                       |                     |         |            |                 |                           |
| Trimethylene glycol                                   | 410                   | 48.843              | 7.553   | 0.684      | 124             | >-35                      |
| n-Caproic acid                                        |                       |                     |         |            |                 |                           |
| 2-Ethylhexanol                                        |                       |                     |         |            |                 |                           |
| Sebacic acid                                          |                       |                     |         |            |                 |                           |
| Tetraethylene glycol                                  | 400                   | 38.570              | 7.955   | 0.591      | 155             | -25                       |
| n-Caprylic acid                                       |                       |                     |         |            |                 |                           |
| C <sub>10</sub> "Oxo" alcohol                         |                       |                     |         |            |                 |                           |
| C <sub>10</sub> -C <sub>11</sub> Alkenylsuccinic acid |                       |                     |         |            |                 |                           |
| Pentamethylene glycol                                 | 470                   | 74.666              | 10.493  | 0.647      | 126             | >-35                      |
| n-Caprylic acid                                       |                       |                     |         |            |                 |                           |
| Methyl alcohol                                        |                       |                     |         |            |                 |                           |
| C <sub>10</sub> -C <sub>11</sub> Alkenylsuccinic acid |                       |                     |         |            |                 |                           |
| Triethylene glycol                                    | 515                   | 62.155              | 9.049   | 0.664      | 125             | >-35                      |
| n-Caprylic acid                                       |                       |                     |         |            |                 |                           |
| Methyl alcohol                                        |                       |                     |         |            |                 |                           |
| C <sub>10</sub> -C <sub>11</sub> Alkenylsuccinic acid |                       |                     |         |            |                 |                           |
| Polyethylene glycol (300 mol. wt.)                    | 390                   | 57.962              | 8.497   | 0.673      | 123             | -30                       |
| n-Butyric acid                                        |                       |                     |         |            |                 |                           |
| Methyl alcohol                                        |                       |                     |         |            |                 |                           |
| Sebacic acid                                          |                       |                     |         |            |                 |                           |
| Tetraethylene glycol                                  |                       |                     |         |            |                 |                           |
| n-Caprylic acid                                       | 360                   | 25.470              | 5.651   | 0.637      | 162             | -15                       |
| C <sub>10</sub> -C <sub>11</sub> "Oxo" alcohol        |                       |                     |         |            |                 |                           |

Lauric acid  
Palmitic acid  
Stearic acid  
Oleic acid  
β-Methoxypropionic acid  
β-Ethoxypropionic acid  
β-Tert.-octoxypropionic acid  
β-Ethylmercaptopropionic acid  
β-Tert.-octylmercaptopropionic acid  
β-Tert.-dodecylmercaptopropionic acid

If desired, various addition agents may be incorporated in the esters of the present invention for the purpose of improving their properties with respect to their usefulness as lubricants. For example, antioxidants, viscosity index improvers, thickeners, pour depressants, dyes, etc., may be added.

Data will be given below showing the properties of several examples of complex esters within the scope of the present invention indicating the adaptability of these esters to lubricating service. All of these esters were prepared by a general esterification method which was carried out in detail as follows: In a 1-liter round bottomed reaction flask, fitted with a reflux condenser and water trap, was placed a charge consisting of 1 mol of dibasic acid, 1 mol of glycol, 4.5 gr. of p-toluenesulfonic acid monohydrate, and 100 ml. of toluene. The mixture was refluxed until exactly one mol of water was collected in the trap. Then, after cooling, 1 mol of monohydric alcohol was added and the reaction continued until no more water collected in the trap. One mol of monobasic acid was then added and the reaction continued until again no

5 The above data indicate that the esters constituting the subject-matter of the present invention possess characteristics, particularly with regard to viscosity index and pour point, which indicate 45 their suitability for general use as lubricating oils and particularly for use where the use of additives is not desirable. The esters of the present invention may also be blended with mineral lubricating oils to give lubricants of improved viscosity index 50 and pour point.

What is claimed is:

1. As a new composition of matter a compound of the formula—



where R is an aliphatic hydrocarbon radical containing 2 to 8 carbon atoms in a straight chain between the —COO— groups; where R' is a radical of the formula —(CH<sub>2</sub>CH<sub>2</sub>O)<sub>n</sub>CH<sub>2</sub>CH<sub>2</sub>—, 65 where n is an integer from 1 to 7; where R'' is an alkyl group containing 1 to 19 carbon atoms; and where R''' is an alkyl group containing 3 to 7 carbon atoms.

2. A composition according to claim 1 in which 70 R is a radical containing 4 carbon atoms.

3. A composition according to claim 1 in which R is a radical containing 4 carbon atoms and R'' is a 2-ethylhexyl radical.

4. A composition according to claim 1 in which 75 R is a radical containing 4 carbon atoms, R'' is a

2-ethylhexyl radical, and R''' is an n-caproyl radical.

5. A composition according to claim 1 in which R' is the radical

—(CH<sub>2</sub>CH<sub>2</sub>O)<sub>2</sub>CH<sub>2</sub>CH<sub>2</sub>—

6. A composition according to claim 1 in which R' is the radical

—(CH<sub>2</sub>CH<sub>2</sub>O)<sub>2</sub>CH<sub>2</sub>CH<sub>2</sub>—

7. A method which comprises reacting one molecular proportion of a polyethylene glycol with one molecular proportion of adipic acid, under conditions which provide for the removal of water formed in the reaction from the reaction zone, until only one molecular proportion of water of reaction is formed and removed, and thereafter adding one molecular proportion of 2-ethylhexanol to the reaction mixture and continuing the

esterification reaction until no more water is formed, and thereafter adding one molecular proportion of n-caproic acid and continuing the esterification reaction until again no more water of reaction is formed.

5 8. A method according to claim 7 in which the glycol employed is triethylene glycol.

PAUL V. SMITH, JR.

10

#### REFERENCES CITED

The following references are of record in the file of this patent:

| UNITED STATES PATENTS |          |               |
|-----------------------|----------|---------------|
| Number                | Name     | Date          |
| 1,786,404             | Young    | Dec. 23, 1930 |
| 2,035,528             | Brubaker | Mar. 31, 1936 |
| 2,073,031             | Sly      | Mar. 9, 1937  |